

## UNITED STATES PATENT OFFICE

2,164,509

COMBUSTION TRAIN ELEMENT AND FUSE  
FOR BLASTING AND PYROTECHNIC AND  
THE LIKE PURPOSES, AND METHOD OF  
PREPARATION THEREOFJames Sinton Bruce Fleming, Ardrossan, and  
Russell Charrosin Payn, Saltcoats, Scotland,  
assignors to Imperial Chemical Industries  
Limited, a corporation of Great BritainNo Drawing. Application August 14, 1936, Serial  
No. 96,118. In Great Britain August 21, 1935

## 11 Claims. (Cl. 52—17)

This invention relates to the preparation of coherent combustion train elements made from a fuse powder, e. g., blackpowder or blackpowder substitutes or constituents thereof, which elements 5 may be used in substitution for blackpowder impregnated cloth and the like for pyrotechnic and similar purposes, in blasting operations, and in the preparation of safety fuse.

The present invention consists in a process for 10 the manufacture of combustion train elements, according to which a fuse powder, e. g., blackpowder or a mixture of ingredients thereof, in finely divided form, is suspended in an aqueous medium saturated with respect to the water-soluble components and is agitated with a proportion of a fibrillated cellulose bonding material, whereupon the suspension is drained to form a wet felt which is then further dried and shaped. The proportion of fibrillated cellulose bonding 15 material is small relative to the weight of the fuse powder or fuse powder ingredients.

By the term fibrillated cellulose bonding material as used herein and in the appended claims we mean cellulose fibrous material which has 20 been beaten or pulped in an aqueous medium in such a manner that the fibres have acquired the crushed or bruised characteristics associated with the product of a blunt beating process. Unbeaten fibrous material, or material which has 25 been beaten with sharp blades so that the individual fibres are merely cut without being crushed, does not usually possess felting properties sufficiently good to justify its use for the purpose of the present invention.

The term fuse powder as used herein and in the 30 appended claims signifies a material which, when in finely divided form, is capable of propagating its own combustion along a train. For the purposes of the invention there may be used blackpowder substitutes, i. e., non-detonating combustible mixtures capable of production in granular or powder form and classifiable in Classes 2 or 4 of the British List of Authorised Explosives, or the ingredients of such blackpowder substitutes. Blackpowder itself, however, and the ingredients of blackpowder are most frequently 35 suitable; and the invention is hereinafter described in relation to blackpowder.

It is convenient that the saturated aqueous 40 solution of the water-soluble constituent of the blackpowder should contain a proportion of alcohol, or other easily evaporated neutral water-miscible organic liquid, in order to depress the solubility of the water-soluble constituent. The 45 water-soluble constituent will usually consist of

potassium nitrate, since blackpowders made with other salts are not usually employed in the manufacture of combustion train elements on account of their hygroscopicity. An unduly high concentration of this ingredient in the solution may militate against proper felting of the fibres, or 5 may have a corrosive effect on metal parts of the apparatus or other undesired effects, but the presence of a proportion of the organic liquid considerably reduces the solubility of potassium 10 nitrate.

In preparing the felt, the finely divided solids and the fibrillated cellulose bonding material are 15 thoroughly mixed and dispersed in the aqueous suspension medium already saturated with the water-soluble constituent, and the material is formed into a felt by filtering, screening or otherwise removing the bulk of the water. The material is advantageously filtered through a screen of fabric or metal gauze. A suitable mesh for 20 the gauze is about 20-100 per linear inch. Some of the remaining moisture may then be removed by pressure or suction and the felt subsequently transferred on a travelling screen or the like to a drying chamber where it is dried off at a suitable temperature such as 40-50° C., being supported by the screen at least until the moisture content has been greatly reduced. For further 25 shaping the felt may be cut or stamped into discs, strips and the like. This should preferably be 30 done while the felt still contains a little moisture, in order to prevent the possibility of ignition as a result of the working of the cutting tool. On the other hand, the material has very little 35 strength until a very considerable proportion of the water has been removed from it. If desired, strips of the substantially dry material may be lightly twisted in order to form a yarn-like element.

The formation of the felt may be carried out 40 with the aid of machinery known in the paper-making art but it may be necessary to provide additional means for agitating the suspension to prevent deposition of the relatively compact and dense noncellulosic particles to the bottom of 45 the reservoir from which the suspension passes to the screen or gauze. Various types and modifications of machinery are suitable for the purpose, for instance cylinder metal machines, or Foudrinier machines. Continuous rotary filters 50 may also be employed. It will be appreciated that the proportion of liquids to solids in the suspension should be chosen with regard to the type of machine employed.

Suitable cellulosic fibrous materials for use in 55

the invention include blunt beaten linters, kraft pulp, esparto, rag and wood pulp. The substantially dry felt prepared from blackpowder containing about 5-15% of its weight of such cellulose fibre is endowed with surprising tenacity and serviceability. Apart from the advantage that shaped pieces may be obtained from it by cutting or the like with great facility, which simplifies the manufacture of pyrotechnic combustion train elements, it has properties which render it suitable for the preparation of a safety fuse.

In the manufacture of safety fuse a strip or yarn of the blackpowder felt is used as the core, around which the covering and counter yarns or other coverings are spun or positioned. In a spinning machine of the usual type, the motion of the covering yarn pulls the core forward with it, so that it is only necessary to enter the end of the length of the fuse element in position.

Combustion train elements prepared from blackpowder dust in accordance with our invention are characterized by a lower burning speed than granular blackpowder or blackpowder dust, while combustion train elements similarly prepared from the unincorporated ingredients of blackpowder have a still lower burning speed. In the manufacture of slow safety fuse, accordingly, the ingredients of the blackpowder may be employed without the expense of the usual operations of incorporation and granulation associated with the manufacture of blackpowder.

Safety fuse may be prepared according to our invention with a slower regular burning speed than any other safety fuse of which we are aware.

Safety fuse of regular burning speed lower than a speed corresponding to 250 seconds per yd. or even lower than one corresponding to 300 seconds per yd. may thus be obtained. It is not claimed however that the safety fuse prepared according to our invention has the property of "spitting" like ordinary safety fuse, and in its application it is usually necessary that the detonator should contain in addition to the usual priming composition a loose charge of a substance which is particularly easy to ignite such for instance as lead dinitroresolate, or lead sulpho-cyanate mixtures. For initiating blackpowder pellets, it is advisable that the fuse should be capped with a perforated cap containing an igniting charge to transfer the ignition from the fuse to the blackpowder. Alternative arrangements for transferring the ignition will be obvious to those skilled in the art.

The proportion of cellulosic fibre present in the felt cannot be indefinitely increased, since the combustion train element will ultimate become uncertain in its propagation combustion. The precise maximum proportion which may be employed will be dependent on a number of factors, including the cross sectional area of the train and the heat capacity of its environment. In the case of safety fuse, in which the element is naturally of small cross sectional dimensions and is surrounded by a considerable amount of heat-absorbing material, a suitable proportion of cellulose fibre is about 5-15% of the total weight, and it is hardly possible to exceed this amount much without adverse effect on the burning properties of the fuse. The use of fibrillated cellulosic material, however, renders it possible to obtain a felt of the requisite strength and coherency with such proportions of cellulose to fuse powder or fuse powder ingredients.

In the manufacture of other types of combustion train element it may be practicable to use

somewhat higher proportions of cellulosic material, e. g., 15% or 20% by weight if desired.

The invention is further illustrated by the following examples in which the parts are parts by weight:

#### Example 1

2000 parts of aqueous alcohol of specific gravity 0.9726 (obtained by mixing water and industrial spirits 66 O. P. in the volumetric proportions 3:1) are saturated with potassium nitrate by the addition of 220 parts of nitrate, and the decanted saturated solution is placed in the stuff chest of a cylinder mould machine provided with paddles to overcome silting. 150 parts in all of the solid ingredients employed in the manufacture of ordinary blackpowder fuse powder are added in such a state of division that they pass through a 60 mesh B. S. sieve and there are also added 180 parts of a blunt beaten suspension of kraft pulp which contains 18 parts of dry kraft pulp and 162 parts of water. A further 18 parts of potassium nitrate are added with the fuse powder ingredients in order to saturate the water introduced into the system in the form of the kraft pulp suspension.

The suspension is well mixed and the wet felt deposited on the cylinder mould is dried down to a moisture content of 10% and the sheet is cut into portions while still containing this percentage of moisture. It is then further dried down to a moisture content of about 1%. The thickness of the sheet is approximately 90 thousandths of an inch.

Long strips of the material may be used either singly or twisted together as fuses or in place of the usual powder core in safety fuse. Discs, or stampings of other suitable shapes, are useful in building up charges in the manufacture of pyrotechnic devices and the like, in which manufacture the operations of weighing out loose charges are replaced by a selection of a suitable number of stampings or pressings from a sheet of the appropriate composition.

#### Example 2

This example illustrates the production of a safety fuse from the sheet prepared as in Example 1. A suitable length of a core portion, consisting of a strip  $\frac{1}{16}$ " wide of the sheet produced according to Example 1, is introduced in place of the core of loose granular blackpowder in a safety fuse machine in which three textile counterings are spun round it in the ordinary way. The fuse is finished in the usual manner.

The burning speed of a fuse made in this way corresponded to 315-325 seconds per yard. For purposes of comparison a fuse similarly fashioned from blackpowder dust in place of the strip of the core material of the present invention was found to have a speed corresponding to 105-110 seconds per yard.

The fuse prepared according to Example 2 was suitable for use with a detonator provided with an auxiliary igniting charge of the lead sulpho-cyanate or lead dinitroresolate type in addition to the usual priming charge and secondary charge.

#### Example 3

The preparation was carried out as in Example 1, except that instead of the ingredients of 150 parts blackpowder there were employed 150 parts of blackpowder dust passing a 60 mesh B. S. sieve. When made up into a safety fuse substitute as described in Example 2, it was found that

the safety fuse had a burning speed corresponding to about 105-110 seconds per yard.

*Example 4*

5 90 parts of blackpowder dust and 100 parts of wet pulped kraft pulp containing 10% of its weight of dry pulp were added to a mixture of 80 parts of water and 20 parts of methylated spirits previously saturated with potassium nitrate and containing sufficient undissolved potassium nitrate to saturate the water added in the form of the pulp. The whole mixture was agitated, screened and dried to form sheets of about 1 mm. in thickness. Before the sheet was quite dried, it was cut into discs. The waste material from the cutting operation is returned to the agitated pulp and reworked. The discs are suitable for use as described in Example 1.

We claim:

20 1. A process of preparing combustion train elements, which comprises suspending a black powder composition in an aqueous medium saturated with respect to the water-soluble components of said composition, agitating said suspension with a relatively small proportion of a fibrillated cellulose bonding material, and removing said aqueous medium to form a felt.

25 2. A process of preparing combustion train elements, which comprises suspending a black powder composition in an aqueous medium saturated with respect to the water-soluble components of said composition, agitating said suspension with 5 to 20% of a fibrillated cellulose bonding material, said percentage being calculated on the weight of the solid content in said suspension, and removing said aqueous medium to form a felt.

30 3. A process of preparing combustion train elements, which comprises suspending a black powder composition in an aqueous medium saturated with respect to the water-soluble components of said composition, agitating said suspension with 5 to 15% of a fibrillated cellulose bonding material, said percentage being calculated on the weight of the solid content in said suspension, and removing said aqueous medium to form a felt.

35 4. A process of preparing combustion train elements, which comprises suspending a black

powder composition in aqueous alcohol saturated with respect to the water-soluble components of said composition, agitating said suspension with a relatively small proportion of a fibrillated cellulose bonding material, removing said aqueous 5 alcohol to form a felt.

5 5. A combustion train element consisting of a coherent felt of burning speed lower than 250 seconds per yard, which felt comprises a black powder composition intermingled with a fibrillated cellulose bonding material.

10 6. A combustion train element consisting of a coherent felt of burning speed lower than 250 seconds per yard, which felt comprises a black powder composition intermingled with from 5 15 to 20% by weight of a fibrillated cellulose bonding material.

15 7. A combustion train element consisting of a coherent felt of burning speed lower than 250 seconds per yard, which felt comprises a black 20 powder composition intermingled with from 5 to 15% by weight of a fibrillated cellulose bonding material.

20 8. A combustion train element consisting of a coherent felt of burning speed lower than 250 25 seconds per yard, which felt comprises unincorporated black powder ingredients intermingled with kraft pulp.

25 9. A process of preparing combustion train elements, which comprises suspending a black 30 powder composition in an aqueous medium saturated with respect to the water-soluble components of said composition, agitating said suspension with a relatively small proportion of a fibrillated cellulose bonding material, removing 35 said aqueous medium to form a moist felt, shaping said felt into the form of a core and enclosing in an envelope.

35 10. A safety fuse including a core of coherent felt of burning speed lower than 250 seconds per 40 yard which felt comprises a black powder composition intermingled with fibrillated cellulose.

40 11. A safety fuse including a core of coherent felt of burning speed lower than 250 seconds per yard which felt comprises a black powder composition intermingled with 5 to 15% by weight of the fibrillated cellulose. 45

JAMES S. B. FLEMING.  
RUSSELL CHARROSON PAYN.